

H. Bessemer.

Making Iron and Steel.

No. 94,996.

Patented Sept. 21, 1869.



Witnesses,

Ch. McAdam  
H. J. Hale

Inventor:

Z. S. Durfee  
atty for Henry Bessemer

# UNITED STATES PATENT OFFICE.

HENRY BESSEMER, OF LONDON, ENGLAND.

## IMPROVEMENT IN THE MANUFACTURE OF IRON AND STEEL.

Specification forming part of Letters Patent No. 94,996, dated September 21, 1869; patented in England; March 21, 1868.

*To all to whom it may concern:*

Be it known that I, HENRY BESSEMER, of Queen Street Place, Cannon street, in the city of London, England, a subject of the Queen of Great Britain, have invented or discovered new and useful Improvements in the Manufacture of Malleable Iron and Steel and in Apparatus used in such Manufacture; and I, the said HENRY BESSEMER, do hereby declare the nature of the said invention, and in what manner the same is to be performed, to be particularly described and ascertained in and by the following statement thereof—that is to say:

These improvements relate, first, to the manufacture of malleable iron and steel from crude molten iron, from remelted pig-iron, and from cast scrap, or other carburets of iron, by means of certain modifications of or additions to the Bessemer process of making malleable iron and steel, such modifications of or additions having for their chief objects the production of cast-steel by a more complete purification of the cheap or inferior kinds of pig or cast iron, and the employment and admixture with such purified inferior iron of molten iron of a more pure or better quality, such as is now generally employed in the Bessemer process.

In carrying my said improvements into practical operation, I prefer to employ a converting-vessel made of stout plate-iron, the vessel being flattened on the two sides where the trunnions are formed. These trunnions I prefer to make of cast-iron, having large ribbed flanges formed thereon, by means of which they are securely fastened to the sides of the vessel, which is much strengthened thereby.

The converting-vessel is provided with two tuyere-boxes, placed at about one-fourth of a circle from each other, so that if the tuyeres in these separate boxes be directed to a point coincident with the trunnions of the vessel, they will be nearly at right angles to each other.

That part of the vessel into which the tuyeres from each box are directed may be hollowed out, or formed into a cavity or hearth; or the tuyeres may simply enter the general curved surface of the interior of the vessel.

I, however, prefer to form two cavities or hearths, separated by a sort of low mound

between them, formed of gannister or other refractory material with which the vessels are usually lined.

By way of distinction, I will call the first or small hearth, A, and the second or larger hearth, B. The first hearth may, if found desirable, be lined or "fettled" with "bull-dog" or with "red ore," as in puddling-furnaces, while the rest of the vessel is lined, by preference, with gannister.

The vessel is provided with suitable openings, as usual, for putting in the fire-clay tuyeres, and also with other openings, *n*, at the sides, for the introduction of an iron bar, to lift up or stir the charge, if necessary.

In some cases I also provide other openings for the insertion of tuyeres or nozzles, for the purpose of injecting certain fluids into the metal, when found desirable, and which will be hereinafter referred to.

The vessel is further provided with a large opening or mouth, for receiving and discharging both the metal and the fuel employed to heat the vessel.

The trunnions of the vessel are so arranged that air or steam may be passed through or around them, and, by means of suitable branch pipes, be conveyed into the tuyere-boxes, as required.

The vessel may be moved on its trunnions by hydraulic apparatus, as at present practiced, or by a small engine, acting on a suitable gearing in connection with the trunnions.

In order that the construction and arrangement of the several parts of the converting-vessel may be fully understood, I have represented the same on the sheet of drawings hereto annexed, where Figures 1, 2, and 3 are vertical sections on the line C D of Fig. 5.

The vessel is shown in side elevation at Fig. 4, and in vertical section at Fig. 5, the section being taken on the line E F of Fig. 4. An end elevation is also shown at Fig. 6.

In these several figures, *a* represents the outer shell of the vessel, made of wrought-iron plates, and *b b* are the cast-iron ribbed trunnion-pates, secured to the sides of the vessel, a part of this casting, at *b\**, being formed into a hollow axis or trunnion, on which the vessel is supported, and on which it moves in suitable bearings *c* formed on the standards *c\**.

The vessel is lined with gannister, or other suitable material, throughout, as shown at *d*; or a part of it may be lined or fettled with bull-dog, red ore, or other materials used to line or fettle puddling furnaces. The vessel is so formed internally as to divide its interior into two hollows or hearths, *A* and *B*, the lining being raised at *d*\*, so as to form a low mound or division between them. Each of these hearths is provided with tuyere-boxes, the hearth *A* having a tuyere-box, *e*, with fire-clay tuyeres *r*, (shown also in plan at Fig. 7,) and the hearth *B* having a tuyere-box, *f*, and tuyeres *s*. (Also shown in plan at Fig. 8.) These tuyere-boxes are both supplied with air from a blast-engine, in the usual manner, by means of the pipes *g* and *h*, which communicate with the hollow axis of the vessel, where stuffing-boxes of the ordinary kind may be employed, and thus admit of the rotation of the vessel on its axis without disconnecting the said pipes. The means of giving axial motion to the vessel are not shown, as the same may be readily accomplished by hydraulic apparatus, as already practiced. The pipe *g*, which conveys air into the tuyere-box *e*, serves also to convey steam thereto, when required, by means of two cocks, one of which communicates with a steam-boiler or steam-supplier, and the other with the reservoir of compressed air, so that during the process either air or steam, or air and steam mixed, may be passed together, at will, through the tuyeres.

The converting-vessel having been heated by blowing up a coke fire, as usual, therein, and the residue of the fuel turned out, the vessel is to be turned into a position suitable for receiving the fluid iron. Some "mill-scales," "hammer-slag," red ore, or any other matters, such as it has hitherto been found desirable to use in puddling iron, may be put into the hearth *A*, and then a charge of molten iron of a cheap or inferior quality may be run in. The position of the vessel at this time is shown at Fig. 3, where it will be observed that the metal *i* is kept below the level of the tuyeres prior to the commencement of the process. A blast of air or steam is then turned on through the tuyeres into the small hearth *A*, and the vessel turned up, so as to cause the molten metal to run into the hearth *A*, as shown in Fig. 2, and be operated upon by the blast.

It must be understood that the tuyeres in the small hearth *A* are of a smaller size and are less in number than is usually employed in the Bessemer process.

As soon as the iron is somewhat raised in temperature, the workman, by means of a suitable valve or cocks, will turn on steam with the air, or he will use steam alone. The result of the partial decarbonization of the metal, by the slow action of a restricted supply of air and the cooling effect of steam operating with the mill-scales and other matters, will tend to convert the metal into a pasty or granular mass, mechanically mixed with fluid

cinder. The constant and somewhat violent heaving up of the mass by the jets of air or steam tends to divide the metal and disseminate it in a more or less granular form throughout the fluid cinder. Additions of mill-scales iron ore, or oxide of manganese, or other substances used to form puddling cinder, may be added, as thought desirable; and if the mass becomes too stiff, an iron bar may be introduced at the openings *n* before named, and the metal thereby raised and divided. Meantime the use of steam may be discontinued and replaced by a blast of air, which will rapidly restore the temperature necessary to carry on the process.

The management of the heat and the employment of air or steam from time to time will thus be left to the judgment and experience of the operator, who will judge of the state of the metal partly by the heavy sound of the escaping blast as it heaves up the metal, and also by the condition of the flame and sparks emitted from the mouth of the vessel.

As soon as the workman judges that the process has been carried far enough, he will turn down the vessel and run therein a charge of molten iron from a neighboring furnace. The iron so added may be a good gray hematite or some other good quality of iron, preferably containing a little manganese and sufficient carbon. He will then turn up the vessel so far that both portions of the metal will run into the second or larger hearth, *B*, as shown at Fig. 1, where the tuyeres and tuyere-holes are larger and more numerous than in the first hearth, so that a powerful blast of air may be driven through the metal and increase its temperature, and completely melt the first charge and unite therewith. The metal may then be run from the vessel into a ladle in the state of steel; but I prefer to entirely decarbonize the double charge of metal before running it from the vessel, and add thereto a known quantity of manganese pig-iron in a fluid state, as commonly practiced in making Bessemer steel.

Although I have herein described how the first portion of the charge, consisting of an inferior iron, may be purified by a process similar in its effects to the process of puddling, I desire it to be understood that the first portion of the charge in the hearth *A* may be, in part, decarbonized and refined by forcing into the fluid metal jets or currents of fluid nitrates of soda or nitrates of potash, or other fluid matters containing or capable of evolving oxygen when brought in contact with molten iron by means of tuyeres or nozzles in the manner fully described in the specification of a patent granted to me in England, No. 965, and bearing even date with this patent, of which this is the specification, my claim to the use of such modes of decarbonizing or purifying crude iron by means of nitrates or chlorates under these Letters Patent being restricted to their employment on a portion only of the metal to be

converted at one time in the vessel, as described.

In order to prevent the rapid wear of furnaces employed in fusing malleable iron or steel on the hearth of such furnaces, I construct the roof and parts most exposed to heat with hollow bricks, or with passages between them, through which I pass a current of air to keep down their temperature, and I also utilize the heat so abstracted by using the heated air to sustain combustion in such furnaces.

In carrying into practical operation this part of my invention, I prefer to mold the bricks of the form shown in Fig. 9, (although many other forms may be used,) the sides of such bricks being tapered as required to form an arch. Their arrangement in the roof of a furnace is shown in Fig. 10, where they form several passages, *m*, which may extend from end to end of the furnace, a current of air being either forced through them or caused to flow through by means of chimney-draft, the cooling effect of which will prevent the bricks from being so rapidly destroyed as would be the case if solid bricks were employed.

My invention also consists in applying the combined action of furnace-heat with the heat developed by jets or currents of air forced into fluid iron, when applied to mixtures of solidified iron or steel with molten carburets of iron, for the purpose of fusing such solid portion and for decarbonizing the same to produce from such mixed materials fluid or malleable iron or steel.

Crude or pig iron of an inferior quality may be more or less purified by puddling, and, either in the state of malleable iron or puddled steel, and in a loose granular condition, or as puddle-balls, may be removed to another suitable furnace; or it may be treated in the furnace in which the puddling process has been carried on. Some molten iron in either case is then added, and a blast of air is driven up through the metal, raising its temperature, and causing, by its joint action with the furnace-heat, the solid portions of the charge to fuse and blend with the rest and pass into the condition of molten malleable iron or steel. When tapped from the furnace it may be mixed with spiegel-eisen or ferro-manganese, and then formed into ingots or other castings.

I also employ the same combined action of jets of air and furnace-heat for the fusion and conversion of wrought scrap-iron of any kind, and other masses of wrought-iron, such as old iron, railway-bars, and also any steel scraps, skulls, spillings, and crep ends of steel rails or forgings. I prefer to employ, for the purposes of this second part of my invention, a reverberatory gas-regenerative furnace, or other gas-furnace in which heated air and gas are used. The jets or currents of air may be forced into the molten metal through movable pipes or tuyeres; but I prefer to employ fixed tuyeres made of fire-clay, and to stop up or cover

over the ends thereof with fire-clay, loam, or gannister previous to turning on the air, the stopping being removed with an iron rod or by the pressure of the air, as may be found most convenient. This mode of treatment is also applicable to iron which has been more or less purified or rendered into steel or malleable iron by the action thereon of nitrate of soda or nitrate of potash, or other substances which yield oxygen on coming in contact with molten iron. Should such metal have become solidified wholly or partially, I render it again fluid by mixing with it molten pig-iron in a furnace heated by fuel, and I also force jets of air into the fluid portion of the mixture; or the process may be conducted in the vessel in which the nitrates or similar substances were applied, the fire-heat and air-jets being used in this vessel.

Having described the several parts of my invention and the manner in which the same may be carried into practical operation, I desire it to be understood that I do not confine myself to the precise details herein given, provided the essential parts of my said improvements be retained; but

What I claim in the manufacture of malleable iron and steel, and in apparatus used in such manufacture, is as follows:

1. I claim the treatment and purification of molten pig or other carburet of iron in a converting-vessel by means of currents of air and steam used separately, or combined and applied in such manner that the metal shall thereby be rendered semi-fluid, pasty, or granular, and become mechanically mixed with the slags or cinder formed in the process, and subsequently the admixture therewith in the same vessel of a further portion of molten pig or other carburet of iron, and the effecting the complete fusion of such metallic mixture into fluid malleable iron or steel by forcing air in sufficient quantities upward through it.

2. I claim the employment of nitrates of soda or nitrates of potash to act on and purify molten pig or other carburet of iron in a converting-vessel, and the subsequent admixture in the same vessel of the iron so treated with another portion of pig or other carburet of iron, and the conversion of such mixture into fluid steel or malleable iron by means of currents of air forced upward through the metal.

3. I claim the construction and employment, in the manufacture of malleable iron and steel, of converting-vessels having two hearths or cavities and separate tuyere-boxes, as herein described.

4. I claim, in the construction of furnaces suitable for fusing malleable iron or steel on the hearths thereof, the use of hollow fire-bricks arranged to form flues or passages, through which currents of air may be caused to pass, as described.

5. I claim the fusion of malleable iron, or steel, or other partially-decarbonized, puddled,

or purified iron on the sole or hearth of a gas or other reverberatory furnace by adding to the materials to be fused a portion of pig-iron or carburet of iron and forcing air into it, so as to cause heat to be generated, which heat, acting in conjunction with the heat of the furnace and by joint action therewith, fuses the solid portions of the metal, and, blending the

mixtures, converts the whole into fluid malleable iron or steel.

HENRY BESSEMER.

Witnesses:

DAVD. S. LONGDON,  
*Catford Hill, Forest Hill.*

G. F. WARREN,  
*No. 17 Gracechurch Street, London, E. C.*